

## UNITED STATES PATENT OFFICE

2,612,455

## SOYBEAN GLUE

Alexander J. Golick, Seattle, Wash., assignor to  
 Monsanto Chemical Company, St. Louis, Mo.,  
 a corporation of Delaware

No Drawing. Application July 23, 1949,  
 Serial No. 106,500.

4 Claims. (Cl. 106—154)

1

This invention relates to an improvement in the wet mixing of soybean glues and to the resulting adhesive. In particular, it discloses a more stable plywood glue obtained by an initial heat treatment of the glue base in the presence of water prior to the addition of the strongly alkaline reagent chemicals required to make the final glue.

The general purpose of the invention is to greatly prolong the useful life of the glue so as to prevent the losses and disadvantages which have attended the objectionably rapid decomposition of soybean glues used hitherto. The present process is broadly applicable to alkaline soybean glues in general and its use is not restricted to any particular reagent formulation.

The soybean glues currently in use for the manufacture of plywood and the like are strongly alkaline colloidal aqueous dispersions obtained by first mixing the soybean material as a heavy bodied suspension in a moderate amount of water to stir out lumps and thoroughly moisten and swell the particles, followed by the addition of further water to insure the desired final consistency along with strong alkalies including hydrated lime, caustic soda, and silicate of soda, usually followed by carbon bisulfide. The final pH always is well above pH 11.5. The final water content of these glues generally ranges between 3 and 4 pounds of water for each pound of original soybean glue base and the desirable viscosity range is usually between about 25 and 150 as measured by the well known MacMichael viscosity determining apparatus using the No. 26 wire. The viscosity of such glues, however, does not remain constant but tends to increase slowly for several hours and then decrease. The decrease in viscosity is attributed to some form of protein decomposition indicated by the fact that, while no ammonia is added as a reagent in making the glue and the odor of ammonia is absent during the period in which the glue is slowly increasing in viscosity, nevertheless an ammoniacal odor becomes progressively evident during the period when the viscosity is decreasing. It is also the experience of the industry that, after any substantial decrease in viscosity and particularly when the odor of ammonia has become evident, the adhesive properties of the glue are greatly diminished and will shortly disappear. Thus, originally normally thick glue, which has thinned with age or developed an ammoniacal odor, has been found to have little or no adhesive power and is worthless.

The rate at which glues of this character decompose varies with time and temperature, de-

2

teriorating most rapidly when mixed with warm water or in a warm room. In any case, glue which has stood overnight is found to have lost either a large proportion or all of its adhesive power. Furthermore, even after three hours, some reduction in viscosity and attendant loss of adhesive power is often evident, particularly in formulations giving an especially high alkalinity or where the water used in making the glue is warmer than the normal 60° F. to 70° F.

This rapid deterioration of soybean glues has always been a troublesome problem in the plywood industry since it compels close correlation between glue making and glue application along with careful planning to make sure that substantially all of the glue will be consumed before deterioration has occurred and especially when the end of the day's run is reached. Also, as noted, there is considerable damage from standard adhesion from the use of glue which has deteriorated.

Thus, it has always hitherto been considered especially important to mix the glue with either cold water or water that is not warmer than normal room temperature and that any use of heat above room temperature is detrimental and likely to cause short glue life with its attendant difficulties.

It has now been discovered that, notwithstanding this long established belief that heat should be avoided in mixing soybean glues, actually the use of heat under proper control is beneficial and, instead of shortening glue life, actually greatly prolongs it, provided heat of the proper intensity and duration is applied in the early stage of the glue making after the soybean material has been mixed up as a suspension in water but before dispersion by the addition of any of the strongly alkaline reagents.

The invention therefore comprises the process and product of the step of initially heating an aqueous suspension of a soybean glue base in the absence of strongly alkaline chemicals for a period of between about 3 and 30 minutes to a temperature in the range between about 120° F. and 212° F. followed by the addition of the customary reagents, whereby the finished glue acquires greatly increased stability and resistance to spontaneous decomposition and loss of adhesive power.

The following example illustrates a preferred embodiment of the invention but is not to be construed in a limiting sense since various modifications which do not depart from the spirit of the invention will be apparent to glue chemists.

*Example*

200 pounds of hot water at about 210° F. is run into the glue mixer followed immediately by the addition during stirring of 100 pounds of soybean flour. The resulting thick aqueous suspension is stirred for about 5 minutes. Then, while the stirring continues, 150 pounds of cold water at a temperature of about 55° F. is added followed by the usual dispersing reagents added successively. These are: 12 pounds of hydrated lime previously suspended in 24 pounds of water, 8 pounds sodium hydroxide previously dissolved in 8 pounds water, 30 pounds of "N Brand" sodium silicate, and finally 2.5 pounds of a mixture of 1.9 pounds of carbon bisulfide dissolved in 0.6 pound carbon tetrachloride, which is added to enhance the water resistance. Stirring of the glue is continued for about 7 minutes whereupon it is ready for use. The resulting dispersed adhesive has an initial MacMichael viscosity of about 50 on the No. 26 wire.

When compared to a similar adhesive made with the same ingredients but with the initial and secondary water added at room temperature (about 70° F.), this new adhesive shows the following differences. The adhesive made with room temperature water has an initial viscosity of about 25 on the No. 26 wire which slowly rises to a peak of about 85 at the end of four hours and then slowly diminishes and, after 24 hours, the adhesive has become thinned to a viscosity of about 10 or less, and has developed a strong odor of ammonia. The adhesive made with hot water also has a slowly rising viscosity curve and reaches a maximum of about 125 at the end of 8 hours with no ammoniacal odor. After standing overnight, it has thinned only slightly and has a viscosity of 100 with only a very slight odor of ammonia. Adhesion tests by making both cold and hot press plywood test panels with both adhesives at various ages show that the adhesive made in the usual way with cold water begins to show noticeable diminution in adhesive power at the end of about 3 hours with a rapid loss of adhesive properties thereafter and, at the end of an overnight period, the adhesive power is entirely lost. The adhesive made as described above with hot water shows adhesive power fully equal to or slightly better than that of the adhesive made with cold water and it is maintained for 7 hours. There is only a very gradual diminution of adhesive strength thereafter and, even when 24 hours old when a slight odor of ammonia is present, the glue is still thick and spreadable and the adhesion is still of borderline commercial character.

The long retention of commercial adhesive power is a new feature not hitherto obtained in soybean glues and particularly the retention of any adhesive power whatever after the odor of ammonia has become detectable is an exception to all previous experience with soybean glues which hitherto have been found to be completely spoiled whenever decomposition has proceeded to the point where the odor of ammonia can be observed.

In regard to the heating procedure and its limitations: it has been found that the remarkable extension of glue life may be obtained by various equivalent heating methods. A heat treatment at about 120° F. appears to be about the minimum which produces an important extension of glue life. At this low temperature, heat treatment for about 30 minutes is desirable. If the heat treatment is obtained as in the foregoing

example by promptly stirring the soybean glue base into water which is close to the boiling point, then the maximum effect may be obtained in as short a time as 3 minutes. Various other methods of applying the heat treatment may, of course, be substituted. For instance, if the glue mixer is provided with a jacket adapted for heating and cooling, the initial water may be added at room temperature and the heat treatment obtained by running steam through the jacket of the mixer during the initial stirring with restricted water which is customary for the elimination of lumps, followed by cooling to room temperature obtained by circulating cold water through the jacket at the end of the heating period.

It has been found to be essential to avoid any substantial heat treatment of the material after the addition of any of the strongly alkaline reagents. If any of these reagents, such as hydrated lime, caustic soda, or sodium silicate, is added while the mixture is very much above room temperature, the chemical activity of such powerful alkaline reagents is naturally greatly enhanced and there is serious danger of alkaline hydrolysis of the protein with resulting loss of adhesive power. However, this restriction does not apply to the presence of small amounts of soda salts producing only a mild alkalinity or of foam depressants such as pine oil which are frequently incorporated in the dry glue base. The pH of the final glue is always well above pH 11.5.

In making glues according to the present invention, the soybean glue base may be used either in the form of meal or flour of various degrees of fineness. Crude extracted soybean meal may be used. If the glue base contains large coarse particles, as in the case of crude extracted soybean meal, the amount of water required to obtain a final glue of the same viscosity will be somewhat increased but the same stabilizing effect from the heat treatment is obtained. The heat treatment also usually causes a slight and unobjectionable increase in viscosity and water requirement in straight soybean flour glues as compared to the same formulations made in the usual way without heat treatment.

The heat treatment may also be applied to so-called soybean blend glues containing mostly soybean material with small amounts of other proteins such as blood or casein as modifying agents. However, since these proteins are thickened or even irreversibly coagulated by extended heating, their presence is permissible in only small amounts and the heating must be shortened and restricted to avoid excessive thickening and increased water requirement. For this reason, the application of the invention is most advantageous with the widely used straight soybean flour glues.

It is a remarkable feature of the present invention that the stabilizing effect of the initial heat treatment of the soybean glue base is always secured regardless of any variations in the reagent formulation used for subsequent conversion of the initial aqueous suspension to the final dispersed adhesive. In all cases, the useful extension of glue life, resistance to decomposition, and delayed appearance of ammoniacal odor are obtained. The full adhesive power is retained for at least 6 hours and there is no ammoniacal odor during that period. In fact, as indicated previously, the adhesive properties of the heat treated adhesive are always as good as or slightly better than those of a corresponding glue made without heat treatment. This holds true even where small amounts of dry powdered soluble soda salts are

mixed with the original dry glue base. The amount of such premixed salts is always very small and their presence does not produce enough alkalinity during the heat treatment to cause any objectionable changes during the heat treatment.

The three strongly alkaline dispersing agents, viz: hydrated lime, caustic soda and sodium silicate—all three of which are always used in soybean glue formulations, are varied somewhat both in amount and order of mixing in various formulations. None of these variations have any adverse effect on the desirable result from the heat treatment. In some formulae, carbon bisulfide, which is normally used to enhance water-resistance, is omitted but its presence or absence is also without effect as far as the extension of glue life due to the heat treatment is concerned.

While no positive explanation can be advanced for the favorable effects of the heat treatment, it appears to have caused some fundamental modification or regrouping of the reactive radicals in the soybean material which, on the one hand, does not have any appreciable effect on the dispersibility or adhesive character but does greatly retard breakdown of the protein. It also seems evident that this change especially retards breakdown of the nitrogenous radicals since, in the heat treated glue, the development of an ammoniacal odor is observed only after very long standing and even then considerable adhesive property is retained.

I claim:

1. In a process of making an aqueous alkaline soybean glue the improvement which consists in mixing a soybean glue base with water to a stirrable consistency in the absence of acidic and strong alkaline reagents and simultaneously stirring the mixture and heat treating it at the range between about 120° F. and 210° F., for between about 3 and 30 minutes, then cooling the mixture to a temperature substantially not in excess of room temperature and adding to the cooled mixture alkaline reagents to form a glue of spreadable consistency.

2. In a process of making an aqueous alkaline soybean glue the improvement which consists in mixing a soybean glue base with water to a stirrable consistency in the absence of acidic and alkaline reagents and simultaneously stirring the

mixture and heat treating it at the range between about 30 minutes at 120° F. and 3 to 5 minutes at 210° F., then cooling the mixture to a temperature substantially not in excess of room temperature and adding to the cooled mixture alkaline reagents to form a glue of spreadable consistency.

3. A glue having a pH of at least 11.5 and a MacMichael No. 26 wire viscosity in the range between about 25 and 150 prepared in accordance with the process of claim 2 and being characterized by the new property of having a slightly ascending viscosity with retention of substantially full adhesive power for a period of at least 6 hours after making with the further feature that during the 6 hour life there is no development of an ammoniacal odor.

4. In a process of making an aqueous alkaline soybean glue the improvement which consists in the step of initially mixing soybean flour to a stirrable consistency with water in the absence of acids and strong alkalies while subjecting the aqueous suspension to heat treatment in the range between about 30 minutes at 120° F. and 3 to 5 minutes at 210° F., then cooling the suspension to a temperature not in excess of room temperature and adding to the cooled suspension strongly alkaline reagents to produce the final adhesive having a pH of at least 11.5 and a MacMichael No. 26 wire viscosity in the range between about 25 and 150.

ALEXANDER J. GOLICK.

#### REFERENCES CITED

35 The following references are of record in the file of this patent:

#### UNITED STATES PATENTS

| Number    | Name        | Date          |
|-----------|-------------|---------------|
| 1,897,469 | Fawthrop    | Feb. 14, 1933 |
| 2,233,439 | Wahlforss   | Mar. 4, 1941  |
| 2,238,329 | Julian      | Apr. 15, 1941 |
| 2,274,983 | Hieronymous | Mar. 3, 1942  |
| 2,350,953 | Bain        | June 6, 1944  |
| 2,361,302 | Little      | Oct. 24, 1944 |

#### FOREIGN PATENTS

| Number  | Country       | Date           |
|---------|---------------|----------------|
| 11,513  | Great Britain | of 1897        |
| 203,969 | Great Britain | Sept. 20, 1923 |